

## UNITED STATES PATENT OFFICE.

JOHN A. GANN, OF MIDLAND, MICHIGAN, ASSIGNOR TO THE DOW CHEMICAL COMPANY, OF MIDLAND, MICHIGAN, A CORPORATION OF MICHIGAN.

## TREATMENT OF LIGHT METAL ALLOYS.

No Drawing.

Application filed January 18, 1927. Serial No. 161,029.

In my copending application, filed Nov. 28, 1921, Ser. No. 518,142, I described an improvement in the art of making alloy articles having magnesium as a principal ingredient and containing one or more metals capable of dissolving in solid magnesium in larger amounts than are found in solution in the alloys as cast, such improvement consisting in subjecting such articles to a heat treatment at 5 a high temperature but below the melting temperature of the most fusible constituent of the alloy. The result of the aforesaid treatment is to cause increased solution of the other metal or metals in the solid magnesium, 10 this being accompanied by a marked increase in the strength and/or plasticity of the articles. The increase in plasticity thus obtained in light metal alloy articles of the class in question is of particular importance 15 where it is desired subsequently to subject the article to plastic deformation, such for example, as to a forging, drawing, rolling, or extruding operation. The articles thus treated are also found to be rendered susceptible to further improvement in certain 20 physical qualities by aging at regulated temperatures.

The improvements herein claimed related to certain specific aspects of the process and 25 resultant product described in my aforesaid application.

In other words, specifically different results may be obtained, depending upon the constitution of the alloy that is subjected to 30 the aforesaid heat treatment, and, while a wider field of use will be found with magnesium-aluminum alloys, other binary as well as ternary and more complex magnesium 35 alloys are susceptible to marked improvement by treatment in the fashion described.

Having regard to the accomplishment of the foregoing and related ends, the invention then consists of the steps hereinafter fully 40 described and particularly pointed out in the claims, the following description setting forth but one of the various ways in which the principle of the invention may be used.

As indicated, above, the principle involved in my improved method of regulated heat 45 treatment is specifically illustrated and described in my co-pending application by reference to a magnesium-aluminum alloy, the one selected by way of example containing from six to eight per cent aluminum. Upon 50 subjecting such an alloy to a high temperature, but below the melting point of the most

fusible constituent of the alloy, this ordinarily being the eutectic, the tensile strength, as well as other physical properties, such as 55 rigidity or plasticity, hardness, etc., may be materially modified and the article rendered more suitable for various mechanical uses as well as adaptable for further fabrication processes.

The improvement obtained in articles subjected to this regulated heat treatment is apparently due to the rearrangement of the micro-structure of the alloy and particularly to an increase in the amount of solid solution 60 of the minor constituent or constituents present at the expense of the eutectic. In other words, the latter, where it includes a properly selected metal or metals, may be caused gradually to dissolve with the result that an increased amount of the metal in question will 65 be found in solid solution in the magnesium.

Even in the case of a magnesium alloy where the minor constituent is a metal such as cadmium, which in casting at once forms a maximum solid solution with the magnesium, 70 heat treatment of the regulated character hereinbefore described may be advantageously employed, inasmuch as it will insure a more uniform distribution of the two metals 75 in such solution, by eliminating cored crystals.

In order to set forth in inclusive fashion, the different types of micro-structure obtainable in cast magnesium alloys, together with the effect of heat treatment of each such type in the fashion hereinbefore described, as also 80 the temperature possibilities for heat treatment of the same, the following tables are herewith presented, the first relating to typical binary magnesium alloys and the second to certain selected ternary and more complex 85 magnesium alloys.

## I. Heat treatment of binary magnesium alloys.

| Type of structure in cast alloy                | Typical alloys          | Effect of heat treatment                                                               | Temperature for heat treatment                                                                                        |
|------------------------------------------------|-------------------------|----------------------------------------------------------------------------------------|-----------------------------------------------------------------------------------------------------------------------|
| 1. Complete solid solution.                    | Mg-Cd                   | Eliminate cored crystals.                                                              | Up to near melting point of solid solution.                                                                           |
| 2. Combination of solid solution and eutectic. | Mg-Al<br>Mg-Zn<br>Mg-Sn | Increase amount of solid solution at expense of eutectic and eliminate cored crystals. | Up to near melting point of eutectic, and when eutectic is all dissolved, up to near melting point of solid solution. |
| 3. Eutectic                                    | Mg-Cu<br>Mg-Ni          | Relieve casting strains; may also cause rearrangement of eutectic.                     | Up to near melting point of eutectic.                                                                                 |

## II. Heat treatment of ternary, etc., magnesium alloys.

| 5  | Type | Composition    | Condition after heat treating. |                        |          |
|----|------|----------------|--------------------------------|------------------------|----------|
|    |      |                | Solid solution                 | Solid soln. + eutectic | Eutectic |
| 10 | 1.   | Mg-Cd-Al*      | Cd+Al                          |                        |          |
|    |      | Mg-Cd-Zn       | Cd+Zn                          |                        |          |
|    | 2.   | Mg-Cd-Al**     | Cd                             | Al                     |          |
|    |      | Mg-Cd-Zn**     | Cd+Al                          | Zn                     |          |
|    |      | Mg-Zn-Al       | Cd+Zn                          | Zn+Al                  |          |
| 15 |      | Mg-Al-Cu       | Zn                             | Al                     |          |
|    |      |                | Zn+Al                          |                        |          |
|    |      | Mg-Cd-Al-Cu    | Al                             | Cu                     |          |
|    |      | Mg-Cd-Zn-Al-Cu | Cd                             | Al                     |          |
| 20 | 3.   | Mg-Cu-Ni       | Cd+Al                          | Zn+Al                  | Cu       |
|    |      |                | Cd+Zn                          | Al                     | Cu       |
|    |      |                | Cd+Zn+Al                       |                        | Cu+Ni    |

\* Al and Zn must be present in small amounts—less than approximately 1% and 0.5% respectively.

\*\* Al and Zn must be present in appreciable amounts—more than approximately 1% and 0.5% respectively.

Other possible combinations of alloying ingredients can be easily formed from the data of Tables I and II above. Four possibilities for obtaining a micro-structure consisting of a solid solution with or without a eutectic by regulated heat treatment, all of which possibilities come under the second type of structure in the foregoing tables, may be noted, viz: (1) binary magnesium alloys with eutectic and solid solution structure still retain after heat treatment both a eutectic and solid solution; (2) binary magnesium alloys with eutectic and solid solution structure lose on heat treatment such eutectic structure, the minor constituent going entirely into solid solution with the magnesium; (3) ternary or more complex magnesium alloys in which at least part of the minor constituents form eutectic with the magnesium and, on heat treatment, one of these constituents is partly or wholly dissolved in the magnesium to form solid solution, while the other or others are present either as solid solution or eutectic; and (4) ternary or more complex magnesium alloys in which at least part of the minor constituents form eutectic with the magnesium and such eutectics have different melting points and vary as to the ease with which they dissolve in the magnesium to form solid solution, and, on heat treatment, one or more of these constituents are partly or wholly dissolved in the magnesium to form solid solution, while the other or others, if any, are present either as solid solution or eutectic.

The differentiation between the foregoing possibilities in some cases is not great; for example, a magnesium-aluminum-zinc alloy not only comes under the third possibility, since it can be so heated that the zinc will dissolve and the aluminum form the basis of the eutectic, but, on the other hand, the same alloy clearly comes under the fourth possibility, since there

is a difference in melting points between magnesium-aluminum eutectic and the magnesium-zinc eutectic, and the aluminum can be present both as solid solution and the eutectic. Again, the magnesium-aluminum-copper alloy will come under both the third and fourth possibilities for there is a difference in melting points between magnesium-aluminum and magnesium-copper eutectics; the magnesium-aluminum eutectic dissolves fairly easily while the magnesium-copper eutectic does not dissolve at all; and the aluminum can be present both as solid solution and eutectic.

The possibilities as to change in structure obtainable by my improved method of heat treatment, where dealing with alloys of the composition coming under the first and third types in the foregoing tables, will it is believed be sufficiently evident from a consideration of the tabulated data without further detailed explanation.

As to the range of temperatures to be employed, this will vary as previously indicated with the composition of the alloy being treated. Thus the maximum temperature should not exceed the melting point of the more fusible constituent which will be the eutectic where present, or the lower melting eutectic if there be more than one. The Mg-Al eutectic, for example melts at 824° F. and where such eutectic occurs, e. g. in an 8% aluminum alloy, a temperature of from 750° to 820° F. will be desirably employed. However, a lower temperature will suffice, provided the heat treatment be sufficiently prolonged. The Mg-Zn eutectic melts at 650° F. and the Mg-Sn eutectic at 1049° F., from which it may be readily ascertained at what temperatures alloys wherein either of these eutectics is present may be most advantageously treated.

Referring to the various possibilities of heat treatment in effecting micro-structural changes in alloys of the second class in Tables I and II above, it will be noted that in my aforesaid copending application in addition to claims of a more comprehensive character, I have claimed specifically the case (being the first possibility hereinbefore explained) where a binary magnesium alloy with eutectic and solid solution still retains after such heat treatment both a eutectic and solid solution. In contradistinction I herein claim the application of such heat treatment to such an alloy where the result is the loss or disappearance of the eutectic structure formed by one of the minor constituents with magnesium (being the second and third possibilities hereinbefore explained). Subordinate to the foregoing, but also distinguishing from such co-pending application, claim is also herein made to the specific case where one of two minor constituents is capable and the other substantially incapable of forming a solid

solution with the magnesium and the heat treatment causes an increased solution of such first-named constituent.

- A typical binary magnesium base alloy to which the present specific method of heat treatment is applicable is one wherein aluminum is the other constituent. If such an alloy, containing for example approximately 8% of the minor constituent is subjected to a heat treatment at from 800° to 820° F. for four hours, or more, the eutectic originally present will have practically if not entirely disappeared, indicating that all of said constituent has gone into solid solution with the magnesium. A typical, more complex alloy is one containing approximately 8.5% of aluminum and 2% of copper, with or without cadmium and/or zinc in still lesser amounts, respectively (e. g. from 0.5-1.0%), the balance being magnesium. Upon heating such an alloy substantially as just described, the aluminum is caused to go from eutectic

into solid solution form, but the eutectic formed of the copper remains, being possibly changed with respect to its arrangement; whereby additional beneficiating results may accrue, as in the relieving of casting strains, etc. Cadmium if included as an ingredient in such last-mentioned alloy will of course be present at all times, i. e., both before and after heat treatment, in the form of a solution; while the zinc, if present initially in an amount sufficiently large to cause it to be included in the eutectic structure, will in general behave in the same manner as the aluminum, noting, however, that its eutectic has a considerably lower melting point and that the heat treatment should accordingly be in graduated stages.

The following tables have been constructed in order graphically to illustrate the effect of my improved method of regulated heat treatment upon allows having the different types of structure hereinbefore set forth, viz:—

### III. Cast structures.



- In the foregoing table, the alloy as cast may have a structure indicated at the starting end of the several arrows or by alloying certain other metals with the alloy having such starting structure result in the structures indicated at the end of the arrows being obtained. As indicated above, there exists a considerable number of possible changes in

structure where different metals constitute the minor alloying constituent or constituents with magnesium forming the base, depending upon the number of such ingredients and the particular metals selected. The following table will serve graphically to illustrate the results obtained by heat treating the structures indicated above, viz:—

### IV. Effect of regulated heat treatment.

| Cast                                                                                                         | Heat treated                                                                                                           |
|--------------------------------------------------------------------------------------------------------------|------------------------------------------------------------------------------------------------------------------------|
| (1) Solid solution + eutectic                                                                                | Solid solution (increased) + eutectic (decreased)                                                                      |
| (2) Solid solution + eutectic                                                                                | Solid solution                                                                                                         |
| (3) { Solid solution + eutectic<br>Eutectic and/or solid solution                                            | { Solid solution (increased) + eutectic (decreased)<br>{ Eutectic and/or solid solution                                |
|                                                                                                              | { Solid solution<br>Eutectic and/or solid solution                                                                     |
| (4 <sup>a</sup> ) { Solid solution + eutectic<br>Solid solution + eutectic                                   | { Solid solution (increased) + eutectic (decreased)<br>{ Solid solution + eutectic                                     |
|                                                                                                              | { Solid solution<br>{ Solid solution + eutectic                                                                        |
|                                                                                                              | { Solid solution<br>{ Solid solution (increased) + eutectic (decreased)                                                |
|                                                                                                              | { Solid solution<br>{ Solid solution                                                                                   |
| (4 <sup>b</sup> ) { Solid solution + eutectic<br>Solid solution + eutectic<br>Eutectic and/or solid solution | { Solid solution (increased) + eutectic (decreased)<br>{ Solid solution + eutectic<br>{ Eutectic and/or solid solution |
|                                                                                                              | { Solid solution<br>{ Solid solution + eutectic                                                                        |
|                                                                                                              | { Solid solution<br>{ Solid solution (increased) + eutectic (decreased)                                                |
|                                                                                                              | { Solid solution<br>{ Solid solution                                                                                   |
|                                                                                                              | { Solid solution<br>Eutectic and/or solid solution                                                                     |

The term "eutectic", as herein used, it will be understood, includes not only the well-known ordinary eutectics with their more or less characteristic lamellar or globular

structure, but also individual more or less well-defined metallic or intermetallic crystals which so often occur with relatively small percentages of added constituents.

Other modes of applying the principle of my invention may be employed instead of the one explained, change being made as regards the composition and method herein disclosed, provided the ingredients or steps stated by any of the following claims or the equivalent of such stated ingredients or steps be employed.

I therefore particularly point out and distinctly claim as my invention:—

- 10 1. In the art of making alloy articles having magnesium as the predominant constituent and also containing as a minor constituent a metal normally forming both a eutectic and a solid solution with the magnesium, the 75 step which consists in subjecting such article to a heat treatment at a high temperature, but below the melting point of such eutectic, to cause substantially complete solution of the latter.
- 15 2. In the art of making alloy articles having magnesium as the predominant constituent and also containing aluminum as a minor constituent in amount sufficient normally to form both a eutectic and a solid solution with the 80 magnesium, the step which consists in subjecting such article to a heat treatment at an elevated temperature, but below the melting point of such eutectic, to cause substantially complete solution of the latter.
- 20 3. In the art of making alloy articles having magnesium as the predominant constituent and also containing as minor constituents a metal capable and another substantially incapable of forming a solid solution with the 85 magnesium, the step which consists in subjecting such an article to a heat treatment at a high temperature, but below the melting point of the most fusible constituent of the alloy, to cause increased solution of such first minor constituent and still leave a definite eutectic structure including such second minor constituent.
- 25 4. In the art of making alloy articles having magnesium as the predominant constituent and also containing aluminum and copper as minor constituents, the step which consists in subjecting such an article to a heat treatment at a high temperature, but below the melting point of the most fusible constituent of the alloy, to cause increased solution of the aluminum in the magnesium and still leave a definite eutectic structure including the copper.
- 30 5. In the art of making alloy articles having magnesium as the predominant constituent and also containing as minor constituents a metal capable and another substantially incapable of forming a solid solution with the 90 magnesium, the step which consists in subjecting such an article to a heat treatment at a high temperature, but below the melting point of the most fusible constituent of the alloy, to cause substantially complete solution of such first minor constituent and still leave a definite eutectic structure including such second minor constituent.
- 35 6. In the art of making alloy articles having magnesium as the predominant constituent and also containing aluminum and copper as minor constituents, the step which consists in subjecting such an article to a heat treatment at a high temperature, but below the melting point of the most fusible constituent of the alloy, to cause substantially complete solution of such first minor constituent and still leave a definite eutectic structure including such second minor constituent.

6. In the art of making alloy articles having magnesium as the predominant constituent and also containing aluminum and copper as minor constituents, the step which consists in subjecting such an article to a heat treatment at a high temperature, but below the melting point of the most fusible constituent of the alloy, to cause substantially complete solution of such first minor constituent and still leave a definite eutectic structure including such second minor constituent. 75

7. As an article of manufacture, a heat treated light metal alloy article, wherein magnesium is the predominant constituent, the alloy containing as minor constituents a metal capable and another substantially incapable of forming a solid solution with the magnesium, such treated article being characterized by having a definite eutectic structure including such second minor constituent and by 80 having an amount of such first minor constituent thus in solid solution in excess of that present in an untreated article of the same composition.

8. As an article of manufacture, a heat treated light metal alloy article, wherein magnesium is the predominant constituent, the alloy containing aluminum and copper as minor constituents, such treated article being characterized by having a definite eutectic 95 structure including the copper constituent and by having an amount of aluminum in solid solution with the magnesium in excess of that present in an untreated article of the same composition. 100

9. As an article of manufacture, a heat treated light metal alloy article, wherein magnesium is the predominant constituent, the alloy containing as minor constituents a metal capable and another substantially incapable of forming a solid solution with the magnesium, such treated article being characterized by having a definite eutectic structure including such second minor constituent and by having an amount of such first minor constituent thus in solid solution in excess of that present in an untreated article of the same composition, such first minor constituent being substantially entirely thus in solution in such treated article. 105

10. As an article of manufacture, a heat treated light metal alloy article, wherein magnesium is the predominant constituent, the alloy containing aluminum and copper as minor constituents, such treated article being characterized by having a definite eutectic structure including the copper constituent and by having an amount of aluminum in solid solution with the magnesium in excess of that present in an untreated article of the same composition, the aluminum being substantially entirely thus in solution in such treated article. 110

Signed by me this 8th day of January, 1927.  
JOHN A. GANN.